

## UNITED STATES PATENT OFFICE

2,233,436

## LUBRICANT

Waldo L. Steiner, Ponca City, Okla., assignor, by  
mesne assignments, to The Lubri-Zol Develop-  
ment Corporation, Cleveland, Ohio, a corpora-  
tion of Delaware

No Drawing. Application January 22, 1940,  
Serial No. 315,126

4 Claims. (Cl. 252—31)

My invention relates to a cutting lubricant in particular, and lubricants generally, and more particularly to a lubricant designed for lubrication of cutting tools and machines for cutting 5 and threading metallic pipes, rods, bolts and the like.

This application is a continuation in part of my co-pending application Ser. No. 62,170, filed Feb. 3, 1936, now Patent No. 2,188,255 of Jan. 23,

10 1940.

Heretofore, cutting lubricants consisted mainly of blends of lubricating oil and a chemical combination of sulphur, usually, with a fatty compound. These early types of cutting oils are 15 fairly satisfactory for most uses but nevertheless have certain distinct disadvantages. Most of them have an objectionable odor and are very dark in color and some are very inefficient. Usually they are rather expensive and difficult to 20 prepare. A great number have an irritating effect on the skin of the operator. Some are extremely viscous when cold and are therefore very unsatisfactory on cold mornings in many shops which are not well heated. Some of the newer 25 cutting lubricants contain sulphur compounds other than those derived from fatty acid derivatives. In all of the above compounds, however, the sulphur is in chemical combination. Furthermore, other things being equal, the efficiency 30 of this type of cutting oil is largely dependent on the instability of the sulphur compound. The more stable the compound the less efficient it is as an aid in cutting and relatively more of it will have to be used for a satisfactory cutting 35 lubricant. On the other hand, if the compound is very unstable, the cutting oil made from it will likely deteriorate in storage.

The object of my invention is to provide an improved cutting lubricant. I have discovered 40 that an improved and superior cutting lubricant may be prepared by blending a petroleum lubricant with a true physical solution of sulphur in certain suitable solvents. My investigation of 45 this new type of cutting lubricant gives sufficient evidence to prove that it is superior to the conventional chemically combined sulphur cutting lubricant in several ways. In the first place, much less sulphur is required to obtain the same efficiency for the lubricant. Secondly, it makes 50 it possible to prepare a cutting lubricant very light in color and quite odorless and one which does not irritate the skin in the slightest degree. Also, they do not congeal at low temperatures. While some old type lubricants containing chemi- 55 cally combined sulphur may be obtained odor-

less, they are invariably dark in color and are usually rather viscous around 30° F.

There are many solvents for sulphur, one of the best being carbon bisulphide. This solvent could not be used commercially in a cutting lubricant because of its high volatility and inflammability. There are other solvents for sulphur to which these objections could not apply which, for other reasons, such as obnoxious odor and insolubility in petroleum oil, I do not prefer. Phenol 10 and aniline are examples. The greatest difficulty in finding a suitable solvent for sulphur for a cutting oil is to discover one which will not allow sulphur to separate out when the mixture is stored at relatively low temperatures. Naturally, 15 a marketable cutting lubricant must be stable under all kinds of possible storage conditions such as might be encountered in winter.

I have found that solutions of sulphur in certain derivatives of naphthalene and similar high 20 boiling aromatic compounds when added to a petroleum lubricant, do not precipitate out sulphur even at very low temperatures when the amount of sulphur is kept within certain limits, and these form the preferred solutions for use in 25 my invention. Naphthalene itself is odoriferous and not very soluble in petroleum oils at low temperatures and, therefore, is not preferred. It is, however, a very efficient solvent for sulphur, especially at high temperatures. Considerable 30 investigation was therefore given to the naphthalene derivatives which are soluble in petroleum at low temperatures. This work led to the discovery that, among the better sulphur solvents 35 which are soluble in petroleum at low temperatures are the chlorine bearing and other halogen bearing derivatives of naphthalene. Furthermore, the best suited of the chlorine bearing derivatives are the penta- and hexa-chloronaphthalenes. These two compounds were found to 40 be able to dissolve more sulphur for a given weight when mixed with a petroleum lubricant than any other solvent investigated, either at high or low temperatures. They have the added desirable properties of being entirely odorless, 45 practically colorless, and quite non-toxic. These two compounds, holding sulphur in solution and dissolved in a petroleum lubricant, will not precipitate out sulphur when stored for several weeks at 0° F. if the sulphur content does not 50 exceed 12 per cent by weight of the chloronaphthalene in the mixture. These chloronaphthalenes are themselves soluble in a petroleum lubricant to the extent of about 10 per cent at 0° F. They are more soluble in the heavier lubricants 55

such as oils having an S. S. U. viscosity of about 250 at 100° F. than in lighter oils having a viscosity of 70 to 100 at 100° F. Thus it is possible to make a cutting lubricant stable to the most 5 adverse storage conditions from these two chloronaphthalenes, containing 1.2 per cent of physically dissolved sulphur. Since sulphur in a physically dissolved state is many times more efficient in a cutting lubricant than when it is 10 in the combined state, this is sufficient to give an excellent and superior cutting lubricant.

Other solvents among the naphthalene derivatives which are satisfactory, but not as efficient as the above two, are as follows in the descending 15 order of their suitability for use in this invention: hepta- and higher chlorine derivatives of naphthalene; mono-, di-, tri-, and tetra-chloro derivatives; decahydronaphthalene (decalin); halogen or chlorine bearing alkylated naphthalenes (methyl, ethyl, amyl, decyl, octadecyl etc.); coal tar oil cut boiling between 400° F. and 600° F. and higher (largely a mixture of alkyl derivatives of naphthalene) and its halogen bearing 20 derivatives; tetralin and other hydrogenated naphthalenes and their halogen bearing derivatives.

Di-alkylbenzenes and similar high boiling alkylated benzenes (one or more alkyl groups) and their halogen bearing derivatives are suitable for 25 this invention but are not as efficient as the naphthalene derivatives. In fact the halogen bearing and chlorine bearing aromatic and alkylated aromatic compounds as a class are usable in my invention.

In preparing a cutting lubricant according to 30 my invention, the following procedure is recommended. The petroleum lubricant is first mixed with the sulphur solvent in the proportion that it is calculated necessary for the amount of sulphur to be held in solution. The mixture is heated to slightly above the melting point of sulphur (or about 250° F.) and the sulphur is then stirred in until all dissolves. No chemical reaction takes place between sulphur and lubricating oil 35 or halogen bearing aromatic derivatives at this temperature and the solution is purely physical. Only a few minutes are required for the solution to take place. Some specific examples of different mixtures of this new type of cutting lubricant 40 with tests to show their value are given, by way of illustration only, and not by way of limitation. The sulphur may also be first dissolved in the sulphur solvent and then (in solution) added to the lubricating oil.

Example No. 1.—A mixture of 80 parts by weight of light lubricating oil and 20 parts by weight of mono-chloronaphthalene was heated to 45 250° F. and one part of sulphur was stirred in until it dissolved. A sample of this mixture stored at 0° F. for several days did not precipitate sulphur. Tested in a 2" thread cutting machine it gave excellent results. The threads were extremely smooth. Its color was very light and its transparency was an aid to the operator in 50 obtaining the best results, thus avoiding a drawback of the dark sulphurated cutting oil containing chemically combined sulphur. On very cold mornings no trouble was encountered from difficulty to flow. A comparison was made between the results obtained with this lubricant and 55 a highly recommended cutting oil containing chemically combined sulphur, which lubricant had a larger amount of sulphur than the lubricant of my invention. The test pipe threaded was 60 a piece of very hard, used, oil well casing. A

number of threads cut with the sulphur-combined lubricant were compared with a number of threads cut with the new type lubricant. The latter threads were appreciably smoother and showed less tearing than the former, thus demonstrating the improved efficiency of a physical solution of sulphur as a cutting lubricant.

Example No. 2.—A mixture of 80 parts by weight of a light petroleum lubricant and 20 parts by weight of coal tar oil (B. P. range 400° F. to 10 580° F.) was heated to 250° F. and one part by weight of sulphur stirred in until it entirely dissolved. This cutting lubricant was used in a 2" thread cutting machine for two months with consistently superior results with respect to the 15 threads obtained while using it.

Example No. 3.—A mixture of 85 parts by weight of petroleum lubricant and 15 parts by weight of decalin was heated to 250° F. and one part by weight of sulphur was dissolved in it. 20 This cutting lubricant when tested in a thread cutting machine gave very satisfactory results.

Example No. 4.—A mixture of 10 parts by weight of penta-chloronaphthalene and 90 parts by weight of a petroleum oil was a viscosity of 25 150 seconds at 100° F. was heated to 250° F. and 30 1 part by weight of sulphur stirred in until dissolved. On testing this mixture for stability at 0° F. for several days, it did not precipitate out sulphur. It was very light and transparent, having a 2 color (A. S. T. M.) and was entirely free of any odor. The cold test was not raised by the addition of the sulphur and chloronaphthalene. When tested on a thread cutting machine it gave 35 results which were superior to any obtained from any cutting lubricant ever tested on this machine.

Considerably less sulphur in the blend than was used in the above examples is sufficient to give a good cutting lubricant. Even as little as .2 per cent sulphur in the blends of my invention gives 40 satisfactory results. Generally, the sulphur content of this type of cutting lubricant should lie between .1 per cent and 2 per cent. More will not be necessary and less will not be entirely satisfactory. The quantity of sulphur to be used is 45 determined by the use to which the cutting oil will be put.

The addition of 1 per cent or 2 per cent of oleic acid to this type of cutting lubricant seems to have 50 a slightly beneficial effect but is not necessary.

This new type of cutting lubricant may be blended with the old sulphur chemical compound type cutting lubricant to improve the latter.

The petroleum lubricants used in the preparation of these cutting oils may be of naphthenic, 55 paraffinic or mixed base source. They may be either raw or refined and should be selected so that the finished lubricant will have a viscosity of 100 to 300 seconds at 100° F. (S. S. U.). Naturally, cutting lubricants with viscosities outside this range may be useful but as a rule are not as satisfactory as those within this range.

Although a cutting lubricant is the primary object of this invention, it is possible to obtain a high class extreme pressure gear lubricant by 60 merely substituting a more viscous hydrocarbon lubricant for the relatively low viscosity oil used in preparing cutting lubricants in the foregoing compositions.

Having thus described my invention, I claim: 70

1. A composition of matter comprising in combination a major proportion of a lubricant and a minor proportion of a physical solution of elemental sulphur in uncombined form dissolved in a minor proportion of a solvent comprising a 75

halogen bearing alkylated aromatic compound which is a sulphur solvent and is itself soluble in said lubricant.

2. A composition of matter comprising in combination a major proportion of a lubricant and a minor proportion of a physical solution of elemental sulphur in uncombined form dissolved in a minor proportion of a solvent comprising a halogen bearing alkylated aromatic compound which is a sulphur solvent and is itself soluble in said lubricant.

3. A composition of matter comprising in combination a major proportion of a lubricant and a minor proportion of a physical solution of ele-

mental sulphur in uncombined form dissolved in a minor proportion of a solvent comprising a halogen bearing alkylated naphthalene which is a sulphur solvent and is itself soluble in said lubricant.

4. A composition of matter comprising in combination a major proportion of a lubricant and a minor proportion of a physical solution of elemental sulphur in uncombined form dissolved in a minor proportion of a solvent comprising a chlorine bearing alkylated derivative of naphthalene which is a sulphur solvent and is itself soluble in said lubricant.

WALDO L. STEINER.